

1

3,795,610  
POWDERY SOFTENING RINSING AGENT  
COMPOSITIONS

Hans-Werner Eckert, Dusseldorf, and Claus Werner, Haan, Germany, assignors to Henkel & Cie GmbH, Dusseldorf, Germany  
No Drawing. Filed Dec. 29, 1971, Ser. No. 213,721  
Claims priority, application Germany, Mar. 24, 1971, P 21 14 129.7

The portion of the term of the patent subsequent to Apr. 24, 1990, has been disclaimed  
Int. Cl. D06m 13/38

U.S. Cl. 252—8.8

4 Claims

### ABSTRACT OF THE DISCLOSURE

A powdery softening rinsing agent composition comprising a combination of (1) an unsaturated carboxylic acid ester of the formula



wherein  $\text{R}_1$  and  $\text{R}_2$  are selected from the group consisting of alkyl and alkenyl having from 10 to 24 carbon atoms,  $\text{R}_3$  is alkyl having 1 to 4 carbon atoms,  $\text{A}$  is selected from the group consisting of alkenyl and alkenylene having from 2 to 5 carbon atoms,  $\text{X}$  is an anion selected from the group consisting of halide and the anion of an organic, non-surface-active acid and  $n$  is an integer of 1 or 2, (2) non-ionic dispersing agents, (3) at least one solid diluent and (4) optionally other customary ingredients of solid softening rinsing agents for washed laundry, where component (1) is present (a) in a homogenous mixture with the other components, or (b) in finely distributed form on the surface of component (3).

### THE PRIOR ART

After the drying of washed textiles, particularly those of cotton or similar cellulose fibers, a distinct hardening or harshening of the handle or hand can be observed. This phenomenon is particularly exhibited if the textiles have been washed in drum-washing machines with a strong mechanical agitation. This undesirable hardening of the textile goods can be avoided, as is well-known, when a softening rinsing agent is added to the last rinsing liquor of the washing process, that conventionally contains cationic compounds with at least two longer-chain alkyl radicals in the molecule. There are liquid softening rinsing agents for laundry on the market which contain as active ingredient difattyalkyldimethylammonium salts, and generally present in the form of an aqueous dispersion. It is known, however, that such cationic softening rinsing agents, even in a strict adherence to the application directions, affect adversely the absorptivity of the treated laundry.

In the copending, commonly-assigned U.S. patent application Ser. No. 146,515, filed May 24, 1971, now Pat. No. 3,729,416 a liquid softening rinsing agent composition is disclosed comprising

(A) From 1% to 25% by weight of an unsaturated carboxylic acid ester of the Formula I



wherein  $\text{R}_1$  and  $\text{R}_2$  are selected from the group consisting of alkyl and alkenyl having from 10 to 24 carbon atoms,  $\text{R}_3$  is alkyl having 1 to 4 carbon atoms,  $\text{A}$  is selected from the group consisting of alkenyl and alkenylene

2

ene having from 2 to 5 carbon atoms,  $\text{X}$  is an anion selected from the group consisting of halide and the anion of an organic, non-surface-active acid and  $n$  is an integer of 1 or 2,

5 (B) From 0.2% to 8% by weight of at least one non-ionic surface-active dispersing agent,

(C) From 0.2% to 30% by weight of at least one water-soluble organic solvent, and

(D) The remainder to 100% by weight of water.

10 The general preparation of the unsaturated carboxylic acid esters of the Formula I is described in U.S. Pat. 3,397,227.

### OBJECTS OF THE INVENTION

15 An object of the present invention is the obtention of powdery softening rinsing agent compositions incorporating the textile softening unsaturated carboxylic acid esters of Formula I which effectively soften washed textiles without an adverse effect on the absorptivity of the treated laundry and which have good dispersibility in cold water.

20 Another object of the present invention is the obtention of powdery softening rinsing agent compositions for washed textiles containing (1) from 1% to 50% by weight of an unsaturated carboxylic acid ester of the formula



25 wherein  $\text{R}_1$  and  $\text{R}_2$  are selected from the group consisting of alkyl and alkenyl having from 10 to 24 carbon atoms,  $\text{R}_3$  is alkyl having 1 to 4 carbon atoms,  $\text{A}$  is selected from the group consisting of alkenyl and alkenylene having from 2 to 5 carbon atoms,  $\text{X}$  is an anion selected

30 from the group consisting of halide and the anion of an organic, non-surface-active acid and  $n$  is an integer of 1 or 2, (2) from 0.2% to 10% by weight of at least one nonionic surface-active dispersing agent, (3) from 0 to 25% by weight of other customary ingredients of solid

35 softening rinsing agents for washed laundry and (4) the remainder up to 100% by weight of at least one solid diluent carrier compatible with rinsing agents for washed laundry, where said unsaturated carboxylic acid ester is present in said composition (a) in a homogenous mixture with the other components or (b) in a finely-divided form on the surface of said at least one solid diluent carrier, and where the particles according to (a) and (b) may be combined as agglomerates.

40 50 These and other objects of the invention will become more apparent as the description thereof proceeds.

### DESCRIPTION OF THE INVENTION

A powdery softening rinsing agent for washed laundry has now been discovered consisting of a combination of esters of unsaturated carboxylic acids of the Formula I



60 wherein

$\text{R}_1$  and  $\text{R}_2$  are alkenyl, or preferably saturated alkyl with 10 to 24, preferably 12 to 20 carbon atoms,

65  $\text{R}_3$  is a lower alkyl with 1 to 4 carbon atoms, particularly methyl,

$\text{A}$  is an alkenyl or alkenylene with 2 to 5 carbon atoms,  $\text{X}^-$  is a halide, particularly chloride or bromide and/or the anion of an organic, non-surface-active acid and

70  $n$  is the number 1 or 2,

with at least one solid diluent for these active substances, nonionic dispersing agents and, optionally, other cus-

tomary ingredients of solid softening rinsing agents for washed laundry, where said esters of unsaturated carboxylic acids, the textile softening active substance, is present in the composition (a) in a homogenous mixture with the other components, or (b) in a finely-divided form on the surface of the solid carrier particles of the diluent, and where the particles according to (a) and (b) may be combined as agglomerates.

In the Formula I, the alkyl radicals  $R_1$  and  $R_2$ , may be straight-chain or branched, and can be, for instance, lauryl, myristyl, cetyl, oleyl, stearyl, arachidyl, behenyl, lignoceryl, etc. Preferred are alkyl radicals  $R_1$  and  $R_2$  which are derived from natural fatty acids, particularly from hardened tallow fatty acids or coconut fatty acids.

Where A is an alkenyl, it can be, for instance, vinyl, allyl, isopropenyl, 1-propenyl, 2-butenyl, 1,3-butadienyl, etc. Where A is an alkenylene, it can be, for instance, vinylene, methylvinylene, 1,4-butadienylene-(1,3), etc. The radical A may be present both in the cis and in the trans form.

As diluents, easily water-soluble or easily, in water dispersible, inert solid carriers, such as, urea, acetamide, biuret, sodium sulfate, solid polyethylene glycols and, optionally, solid forms of the below listed souring- and sequestering agents come into consideration. The other ingredients of the powdery softening rinsing agents for laundry of the invention are particularly nonionic dispersing agents as well as, optionally, optical brighteners, antimicrobial active substances, souring- and sequestering agents, perfumes and dyes, etc.

The powdery agents of the invention are present as powders, agglomerates or granulates. A particle size of from 0.1 to 3 mm. is desirable, preferably at least 70% of the particles should be from 0.3 to 2 mm. The term "powdery" is used here in its general meaning, as is it usually employed in connection with textile auxiliaries, so that particle sizes from a fine powder to coarse grains including granulates are included.

The agents of the invention are distinguished by a good dispersibility in cold water. With the treatment of washed laundry by the softening rinsing agents for laundry of the invention, fabrics hardened by washing, particularly cotton terry cloth, become soft and nappy. Particularly advantageous, in comparison to known cationic softeners, is the practically insignificant effect on the absorptivity of these fabrics. The softening rinsing agents for washed textiles of the invention render, therefore, the fabric hardened by washing, particularly cotton terry cloth, again agreeably soft and nappy. Such treated fabrics possess, in comparison to the untreated washing goods, only a slightly diminished absorptivity and in comparison to the washing goods treated with known cationic softeners, a substantially improved absorptivity. In addition, by the treatment with the agents, according to the invention, an undesirable static charging of the textiles, particularly those of synthetic fibers, is largely prevented.

The powdery agents of the invention are utilized in such amounts that the concentration of the textile softener of Formula I is in the range of from 0.1 to 2.0, preferably from 0.2 to 1.0 gm./l. of the aqueous treatment liquor.

The composition of the powdery softening rinsing agents for laundry of the invention lies generally in the range of the following formulation based on the anhydrous substances:

1% to 50%, preferably 5% to 25% by weight of carboxylic acid esters of the above defined Formula I, 0.2% to 10%, preferably 1% to 6% by weight of nonionic dispersing agents, 0 to 25%, preferably 0.3% to 15% by weight of other customary ingredients of softening rinsing agents for laundry, remainder, solid carriers from the group of urea, acetamide, biuret, sodium sulfate, solid polyethylene glycols,

Of the other customary ingredients of solid softening rinsing agents for laundry at least one of the following components may be present, in the stated amount, based on the whole composition:

- 5 0.01% to 5.0% by weight of antimicrobial active substance,  
10 0.1% to 10.0% by weight of souring and sequestering agents,  
10 0.01% to 0.8% by weight of cotton brighteners,  
0.01% to 0.8% by weight of polyamide brighteners,  
0.01% to 0.8% by weight of perfume,  
0.00001% to 0.08% by weight of dye.

The active softening ingredients of Formula I, used according to the invention, can be prepared in a known, not claimed herein, manner. The compounds of Formula I may be obtained by the reaction of the alkali salts of the unsaturated carboxylic acids with 3-chloro-2-hydroxy-propyltrialkyl-ammonium halide or by the reaction of the unsaturated carboxylic acid with glycidyl-trialkyl-ammonium halide. In addition, the compounds may be obtained from the unsaturated carboxylic acid, an epihalohydrin, for instance, epichlorohydrin, and a tertiary amine by reaction in an inert solvent.

25 The particularly preferred compounds of the Formula I are the esters of acrylic, methacrylic and crotonic acids, 3-butene carboxylic acid and 3-methyl-3-butene carboxylic acid, as well as of maleic, fumaric, itaconic, mesaconic, methylenemalonic, citraconic, muconic acids, etc.

30 As carboxylic acid ester of the Formula I, for instance, the following may be used:

- (1) Acrylic acid ester of [2-hydroxy-3-(di-hexadecyl-methyl-ammonium)-propyl] chloride;  
35 (2) Acrylic acid ester of [2-hydroxy-3-(dicocoalkyl-methyl-ammonium)-propyl] chloride;  
(3) Methacrylic acid ester of [2-hydroxy-3-(di-tetradecyl-methyl-ammonium)-propyl] chloride;  
40 (4) Crotonic acid ester of [2-hydroxy-3-(di-hexadecyl-methyl-ammonium)-propyl] chloride;  
(5) Crotonic acid ester of [2-hydroxy-3-(ditallowalkyl-methyl-ammonium)-propyl] chloride;  
45 (6) Acrylic acid ester of [2-hydroxy-3-(di-tallowalkyl-methyl-ammonium)-propyl] chloride;  
(7) Crotonic acid ester of [2-hydroxy-3-(di-cocoalkyl-methyl-ammonium)-propyl] chloride;  
(8) Maleic acid bis-ester of [2-hydroxy-3-(di-dodecyl-methyl-ammonium)-propyl] dichloride;  
50 (9) Maleic acid bis-ester of [2-hydroxy-3-(di-cocoalkyl-methyl-ammonium)-propyl] dichloride;  
(10) Maleic acid bis-ester of [2-hydroxy-3-(di-tallowalkyl-methyl-ammonium)-propyl] dichloride;  
55 (11) Fumaric acid bis-ester of [2-hydroxy-3-(di-dodecyl-ethyl-ammonium)-propyl] dichloride;  
(12) Furmaric acid bis-ester of [2-hydroxy-3-(di-cocoalkyl-methyl-ammonium)-propyl] dichloride;  
60 (13) Itaconic acid bis-ester of [2-hydroxy-3-(di-dodecyl-methyl-ammonium)-propyl] dichloride;  
(14) Muconic acid bis-ester of [2-hydroxy-3-(di-tetradecyl-methyl-ammonium)-propyl] dichloride.

The compounds of the Formula I are obtained, as already mentioned, in the preparation generally as halides, particularly as chlorides and bromides. Preferably, the compounds of the Formula I are also incorporated into the agents of the invention as halides. However, in mixture with other ingredients of the agents, at least part of the halide anions may be replaced by other acid radicals which are generally admixed into the preparations of the invention as alkali metal salts and present in this form, conventional ingredients of the softening rinsing agents for washed textiles.

The carboxylic esters of the Formula I, to be used according to the invention, are mostly present as oily, pasty or waxy substances. Their consistency depends widely

upon the length and degree of saturation of the radicals  $R_1$  and  $R_2$ ; also whether the radicals  $R_1$  and  $R_2$  possess a homogenous chain length or if they are present as technical mixtures of homologs. These solid to oily active substances are readily converted to powdery products when they are suitably admixed with the named solid carriers.

The invention relates further to processes for the preparation of powdery softening rinsing agents for laundry of the above given composition.

According to a first process, the preparations of the invention are obtained by spraying the active substance of the Formula I in the temperature range of from 20° C. to 80° C. onto a moving bed of the solid carriers together with the nonionic dispersing agents and, optionally, other customary ingredients, particularly optical brighteners, in a liquid mixture with water and/or volatile organic solvents from the group of methanol, ethanol, isopropanol, acetone, methylene chloride, chloroform.

In this method, preferably, carriers are used with a surface as large as possible and a low bulk weight, for instance a bulk weight of from 100 to 700 gm./l. Products of such bulk weight are obtained, for instance, by calcination of crystal-water containing inorganic salts, particularly of sodium sulfate.

Another preparation process for the agents of the invention is characterized in that an aqueous mixture of the ingredients, which are preferably present in a concentration of from 15% to 35% by weight, is heat-dried at temperatures above 100° C., preferably in the range of from 105 to 125° C.

According to a preferred variant of this process, the heat-drying is carried out by pouring of the aqueous mixture in a thin layer onto hot surfaces. Another preferred variant is characterized in that the heat-drying is effected by spraying of the aqueous charge into a hot gas stream.

In all cases, the powder properties of the process products may be improved by incorporation of slight amounts of substances with a large surface, such as microcrystalline silicic acid, magnesium silicate, etc.

The preparations of the invention produced by the named processes, particularly by the methods of heat-drying, are distinguished by good pourability and good storability, dustlessness and by quick dispersibility in cold water. Insofar the preparations of the invention contain temperatures sensitive or volatile ingredients, such as the below-named antimicrobial or perfumes, they are added to the finished powder.

In the following, the ingredients contained in the softening rinsing agents for washed textiles of the invention, are described more particularly by their various classes.

As nonionic dispersing agents, as they may be contained in the agents of the invention, nonionic surface-active agents are particularly suited, here designated in the following as "nonionics." These are products which owe their hydrophilic properties to the presence of polyether chains, amineoxide, sulfoxide or phosphine oxide groups, alkylolamide groups as well quite generally to an excess of hydroxyl groups. Such nonionics contain in the molecule at least one hydrophobic radical of 8 to 26, preferably 10 to 20 and particularly 12 to 18 carbon atoms and at least one nonionic water-solubilizing group. The preferably saturated hydrophobic radical is mostly of an aliphatic, optionally also alicyclic nature. It can be connected directly to the hydrophilic groups or over connecting members. As connecting member, for instance, benzene rings, carboxylic acid ester or carbonamide groups, ether-like or ester-like bound radicals of polyhydric alcohols, such as those of the ethylene glycol, the propylene glycol, the glycerine or of corresponding polyether radicals, are of interest.

Of particular practical interest are the products obtained by addition of ethylene oxide and/or glycidic to fatty alcohols, alkylphenols, fatty acids, fatty amines, fatty acid or sulfonic acid amides having the above hydro-

phobic radicals. These nonionics may contain from 4 to 100, preferably 6 to 40 and particularly 8 to 20 ether groups, above all ethylene glycoether groups, per molecule, in addition, in these polyether chains or at their end, propylene or butyleneglycoether groups or polyether chains may be present.

To the "nonionics" further belong the products, known under the trade name "Pluronics" or "Tetronics." They are obtained from water-insoluble polyoxypropylene glycols of from water-insoluble propoxylated lower aliphatic alcohols, containing 1 to 8, preferably 3 to 6 carbon atoms, or from water-insoluble propoxylated alkylene diamines. These water-insoluble (that is hydrophobic) propylene oxide derivatives are transformed by ethoxylation to give water-solubility and come under the named nonionics." Finally, as "nonionics," "Ucon-Fluid" which are partly still watersoluble reaction products of the above-named aliphatic alcohols with propylene oxide, are useable.

In addition, the fatty acid or sulfonic acid alkylolamides which are derived, for instance, from mono or diethanolamine, from dihydroxypropylamine or other polyhydroxyalkylamines, for instance the glycamines are in the class of useable "nonionics."

To the surface-active amine oxides belong, for instance, the products derived from higher tertiary amines containing one hydrophobic alkyl aradical and two shorter alkyl and/or alkylol radicals with up to 4 carbon atoms.

As nonionic dispersing agents, optionally suitable are non-surface-active, water-soluble or water-emulsifiable or dispersible compounds, such as partial fatty acid glycerides as well as such compounds which contain no hydrophobic radicals in the sense of the above-described nonionic surface-active agents, such as polyethylene glycols, ethylene oxide adducts of glycerine and other polyalcohols, etc.

Inorganic and non-surface-active organic acids, innocuous to the fibers to be treated, with 1 to 8 carbon atoms are suitable as souring and sequestering agents, such as amidosulfonic acid, urea compounds of orthophosphoric acid, boric acid, oxalic acid, lactic acid, glycolic acid, citric acid, tartaric acid, benzoic acid, phthalic acid, glutamic acid, acetic acid and propionic acid as well as benzene, toluene or xylene sulfonic acids, sulfoacetic acid or sulfobenzoic acids.

Mono or polycarboxylic acids or hydroxycarboxylic acids or their water-soluble salts from the group of the oxalic acid, lactic acid, glycolic acid, citric acid, tartaric acid, luconic acid, malonic acid are in the class of sequestering agents.

Anti-microbial active substances are here understood as bactericidal or bacteriostatic or fungicidal or fungistatic acting compounds. These active substances should be water-soluble as such, or in the form of their salts. The anti-microbial active substances, useable according to the invention, are mostly quaternary ammonium compounds, particularly those which contain, in addition to a long-chain aliphatic and two short-chain aliphatic hydrocarbon radicals, an organic radical in the molecule, either aromatic residue connected over an aliphatic carbon atom to the nitrogen atom or an aliphatic residue with double bonds. Examples for such anti-microbial quaternary ammonium compounds are the following:

dimethyl-benzyl-dodecyl-ammonium chloride,  
dimethyl-benzyl-tetradecyl-ammonium chloride,  
dimethyl-(ethylbenzyl)-dodecyl-ammonium chloride,  
dimethyl-benzyl-decyl-ammonium bromide,  
diethyl-benzyl-dodecyl-ammonium chloride,  
diethyl-benzyl-octyl-ammonium chloride,  
dibutyl-allyl-, methyl-ethyl-benzyl-,  
ethyl-cyclohexyl-allyl- and ethyl-crotyl-diethylamino-  
ethyl-,  
dodecyl-ammonium chlorides.

Other usable antimicrobial active substances are the lower alcohols or diols, substituted both by bromine and nitro groups, with 3 to 5 carbon atoms, such as the compounds 2-bromo-2-nitro-propanediol-1,3, 1-bromo - 1 - nitro-3,3,3-trichloropropanol-2, 2-bromo - 2 - nitro-butanol-1.

As anti-microbial active substances, also suitable are phenolic compounds of the type of the halogenated phenols with 1 to 5 halo substituents, particularly chlorinated phenols; alkyl-, cycloalkyl-, aralkyl- and phenyl-phenols with 1 to 12 carbon atoms in the alkyl radical and with 1 to 4 halo substituents, particularly chlorine and bromine in the molecule; alkenyl bis-phenols, particularly derivatives substituted by 2 to 6 halogen atoms and optionally by lower alkyl or trifluoromethyl groups with an alkylene bridge consisting of 1 to 10 carbon atoms; hydroxy benzoic acids or their esters and amides, particularly anilides which may be substituted in the benzoic acid and/or aniline radical especially by 2 or 3 halogen atoms and/or trifluoromethyl groups; o-phenoxyphenols which may be substituted by 1 to 7, preferably 2 to 5 halogen atoms and/or the hydroxyl, cyano, carbome-thoxy, and carboxyl group or by lower alkyl. A particularly preferred derivative of the class of o-phenoxyphenols is 2-hydroxy-2',4,4'-trichlorodiphenyl ether.

The usable brighteners are mostly, if not exclusively, derivatives of aminostilbene-sulfonic acid or diaminostilbene-sulfonic acid, diarylpyrazolines, carbostyryls, 1,2-di-(2-benzoxazolyl)- or 1,2-di-(2-benzimidazolyl)-ethylenes, benzoxazolyl-thiophens, and of the coumarins.

Examples for brighteners from the class of the derivatives of the diaminostilbene sulfonic acid are compounds according to Formula II:



In the formula, R<sub>1</sub> and R<sub>2</sub> signify alkoxy groups, amino groups or residues of aliphatic, aromatic or heterocyclic, primary or secondary amines, or residues of aminosulfonic acids, while aliphatic residues present in the above groups preferably contain 1 to 4, and especially 2 to 4 carbon atoms, and in the heterocyclic ring systems, five- or six-membered rings are usually of interest. Aniline, anthranilic acid or anilinesulfonic acid residues are preferred as the aromatic amines. Brighteners derived from diaminostilbenesulfonic acid are mostly used as cotton brighteners. The following products derived from the above Formula II in which R<sub>1</sub> represents the residue —NH—C<sub>6</sub>H<sub>5</sub> and R<sub>2</sub> may represent the following residues, are at present on the market.



Some of these brighteners are to be regarded as transitional types to the cotton brighteners as regards their affinity for the fiber, for example the brightener in which R<sub>2</sub> equals —NH—C<sub>6</sub>H<sub>5</sub>. The compound 4,4'-bis-(4-phenyl-1,2,3-triazolyl-2-)-stilbenedisulfonic acid-2,2' also belongs to the cotton brighteners of the diaminostilbene-sulfonic acid type.

Diarylpyrazolines of Formulas III and IV belong to the polyamide brighteners,



10



In Formula III, R<sub>3</sub> and R<sub>5</sub> represent hydrogen atoms, or alkyl or aryl residues possibly substituted by carboxyl, carbonamide or ester groups.

15 R<sub>4</sub> and R<sub>6</sub> represent hydrogen or short-chain alkyl residues.

Ar<sub>1</sub> and Ar<sub>2</sub> represent aryl residues such as phenyl, diphenyl or naphthyl, which may carry further substituents such as hydroxy, alkoxy, hydroxyalkyl, amino, alkyl-amino, acylamino, carboxyl, carboxylic acid ester, sulfonic acid, sulfonamide and sulfone group or halogen atoms.

Brighteners of this type found at present on the market are derived from the Formula IV, and the residue R<sub>7</sub> may represent the groups Cl, —SO<sub>2</sub>—NH<sub>2</sub>, —SO<sub>2</sub>—CH=CH<sub>2</sub> and —COO—CH<sub>2</sub>—CH<sub>2</sub>—O—CH<sub>2</sub>, while the residue R<sub>8</sub> in all cases represents a chlorine atom. 9-cyano-anthracene is also on the market as a polyamide brightener.

In addition, aliphatic or aromatic substituted amino-coumarins belong to the polyamide brighteners, for example, 4-methyl - 7 - dimethylamino- or 4-methyl-7-diethylamino-coumarin. Further useful polyamide brighteners are the compounds 1-(benzimidazolyl-2')-2-(1-hydroxyethyl-benzimidazolyl-2')-ethylene and 1-ethyl-3-phenyl-7-diethylamino-carbostyryl. Suitable brighteners for polyester

35 and polyamide fibers are the compounds 2,5-di-(benzoxazolyl-2')-thiophene and 1,2-di-(5'-methyl-benzoxazolyl-2')-ethylene.

#### EXAMPLES

40 The following examples describe the preparation of some powdery softening rinsing agents for laundry, according to the invention. The same, however, are not to be deemed limitative of the invention in any respect.

#### EXAMPLE 1

45 20.0% by weight of the acrylic acid esters of [2-hydroxy-3-(N,N-di-hexadecyl - N - methylammonium)-propyl] chloride,

2.0% by weight of glycolic acid (100%),

50 3.0% by weight of the adduct of nonylphenol with 9 to 10 mols of ethylene oxide

15.0% by weight of sodium sulfate (anhydrous),

60.0% by weight of urea

The softening rinsing agent for laundry was prepared 55 as follows: The textile softener and the nonionic dispersing agent were melted to a homogenous mixture at 50° C. to 60° C. Simultaneously, the organic acid and the carriers were dissolved in water, preheated to 50° C., and the above-named melt was stirred into this solution. The

60 amounts were utilized so that 1 kg. of all the ingredients of the softening rinsing agent of above composition was allotted to 5 liters of water. The dispersion thus obtained was atomized in a spray tower at 105° C. A white, fine-grained and good pourable powder resulted. To the finished preparation perfumes and anti-microbial active substances may be added.

The textile softener, the acrylic acid ester of [2-hydroxy-3-(N,N-di-hexadecyl-N-methylammonium)-propyl] chloride, used according to Example 1, can be prepared by the following procedure, according to U.S. Pat. 3,397,227.

70 480 gm. (1.0 mol) of N,N-di-hexadecyl-methylamine and 90 gm. (1.25 mols) of acrylic acid were dissolved in 1 liter of isopropyl alcohol and 116 gm. (1.25 mols) of epichlorohydrin as well as 0.5 gm. of 2,6-di-tert.-butyl-4-

methylphenol as inhibitor were added to this solution. After heating for 24 hours at 60° to 65° C., the solvent and excess starting material were distilled off in vacou. The obtained product may be used wtihout further purification.

The other active textile softening ingredients of the Formula I are obtained in an analogous manner.

#### EXAMPLE 2

20.0% by weight of themethacrylic acid ester of [2-hydroxy-3-(N,N-ditetradecyl-N-methylammonium) - propyl] chloride,  
2.0% by weight of glycolic acid (100%),  
3.0% by weight of the adduct of nonylphenol with 9 to 10 mols of ethylene oxide,  
37.5% by weight of sodium sulfate (anhydrous),  
37.5% by weight of urea.

The softening rinsing agent for laundry according to Example 2 was prepared as follows:

400 gm. of the textile softener, 60 gm. of the non-ionic dispersing agent and 40 gm. of glycol acid were mixed at 55° C. with 200 ml. of water and 350 ml. of isopropanol. The liquid mixture was sprayed at this temperature with the aid of a spraying apparatus into a rotating drum and onto the powdery carrier substances. The latter consisted of a mixture of 750 gm. of calcinated sodium sulfate of a bulk weight of 460 gm./l. and 750 gm. of urea of a bulk weight of 485 gm./l. After the spraying, the product mixture was agitated for another 10 minutes in the drum. The other specified products, according to 30 the invention, can also be prepared by this method.

#### EXAMPLE 3

18.2% by weight of the methacrylic acid ester of [2-hydroxy-3-(N,N-ditetradecyl - N - methylammonium-propyl] chloride,  
1.8% by weight of glycolic acid (100%),  
2.7% by weight of the adduct of nonylpehnl with 9 to 10 mols of ethylene oxide,  
9.1% by weight of sodium sulfate (anhydrous),  
68.2% by weight of urea.

The softening rinsing agent for laundry, according to Example 3, was prepared as follows:

The textile softener and the non-ionic dispersing agent were melted together at 50° C. to 60° C. to a homogenous mixture and simultaneously glycolic acid, sodium sulfate and urea were mixed at 50° C. with a 2½-fold amount of water. The above named melt was stirred into this mixture and the slurry, thus obtained, was brought onto a roller-drier, whose rolls had a temperature of 140° C. The product, after evaporation of water, was formed as a thin solid layer, that was lifted off the rolls in the form of scales. The scales were converted into a powder by grinding. The other specified preparations, according to the invention, can also be prepared by this method.

#### EXAMPLE 4

20.0% by weight of the maleic acid bis-ester of [2-hydroxy-3-(N,N-didodecyl - N - methylammonium)-propyl] chloride,  
2.0% by weight of glycolic acid (100%),  
3.0% by weight of the adduct of cetyl-oleyl alcohol with 10 mols of ethylene oxide,  
15.0% by weight of sodium sulfate (anhydrous),  
60.0% by weight of urea.

#### EXAMPLE 5

20.0% by weight of the methacrylic acid ester of [2-hydroxy-3-(N,N-ditetradecyl - N - methylammonium)-propyl] chloride,  
2.0% by weight of glycolic acid (100%),  
2.9% by weight of the adduct of a fatty alcohol (C<sub>12</sub>-C<sub>18</sub>) with 4 mols of ethylene oxide,

0.1% by weight of a cotton brightener of Formula II, in which R<sub>1</sub> is anilino and R<sub>2</sub> is dihydroxyethylamino, 15% by weight of sodium sulfate (anhydrous), 60.0% by weight of urea.

5 Examples 4 and 5 can be prepared by any of the methods specified in Examples 1 to 3.

The powdery softening rinsing agents for laundry of the invention, according to Examples 1 to 5, are distinguished by a quick distribution and dispersion in cold water, so that the effect of the textile softener at its use in the last rinsing cycle of a washing machine is complete. The treatment with the preparations of the invention leads already at an application concentration of 0.5 gm. of the textile softener per liter of rinsing liquor to a full and soft hand of hardened fabric. The soft-rinsed fabrics possess also a good absorptivity.

The preceding specific embodiments are illustrative of the practice of the invention. It is to be understood, however, that other expedients known to those skilled in the art, or disclosed herein, may be followed without departing from the spirit of the invention or the scope of the appended claims.

We claim:

25 1. Powdery softening rinsing agent compositions for washed textiles consisting essentially of (1) from 1% to 50% by weight of an unsaturated carboxylic acid ester of the formula



40

wherein R<sub>1</sub> and R<sub>2</sub> are selected from the group consisting of alkyl and alkenyl having from 10 to 24 carbon atoms, R<sub>3</sub> is alkyl having 1 to 4 carbon atoms, A is selected from the group consisting of alkenyl and alkenylene having from 2 to 5 carbon atoms, X is a halide anion and n is an integer of 1 to 2, (2) from 0.2% to 10% by weight of at least one non-ionic surface-active dispersing agent selected from the group consisting of a water-soluble dispersing agent and a water-dispersible dispersing agent, and (3) the remainder up to 100% by weight of at least one solid diluent carrier compatible with rinsing agents for washed laundry selected from the group consisting of easily water-soluble compounds and easily, in-water-dispersible compounds, where said unsaturated carboxylic acid ester is present in said composition (a) in a homogeneous mixture with the other components, or (b) in a finely-divided form on the surface of said at least one solid diluent carrier, and where the particles according to (a) and (b) may be combined as agglomerates, and where the particle size in said composition ranges from 0.1 to 3 mm. and at least 70% of the particles in said composition have a particle size of from 0.3 to 2 mm., whereby said composition has good dispersibility in cold water.

60 2. The powdery softening rinsing agent compositions of claim 1 wherein said solid diluent carrier compatible with rinsing agents for washed laundry is an inert easily-water-soluble or easily-water-dispersible solid carrier selected from the group consisting of urea, acetamide, biuret, sodium sulfate and solid polyethylene glycols.

70 3. The powdery softening rinsing agent composition of claim 1 wherein component (1) is present in an amount of from 5% to 25% by weight, and component (2) is present in an amount of from 1.0% to 6.0% by weight.

4. The powdery softening rinsing agent compositions of claim 1 containing at least one of the following ingredients in the amounts specified:
- from 0.01% to 5% by weight of antimicrobial active compounds,  
 from 0.1% to 10% by weight of souring and sequestering agents,  
 from 0.01% to 0.8% by weight of cotton optical brighteners,  
 from 0.01% to 0.8% by weight of polyamide optical brighteners,  
 from 0.01% to 0.8% by weight of perfumes, and  
 from 0.00001% to 0.08% by weight of dyes.

## References Cited

## UNITED STATES PATENTS

|           |        |                |           |
|-----------|--------|----------------|-----------|
| 3,573,091 | 3/1971 | Waldman et al. | 117—100   |
| 3,637,495 | 1/1972 | Eckert et al.  | 252—8.8   |
| 3,329,706 | 7/1967 | Sobolev        | 260—485 X |
| 3,397,227 | 9/1968 | Sobolev        | 260—486   |

HERBERT B. GUYNN, Primary Examiner

U.S. Cl. X.R.

117—139.5 C. Q.